

## UNITED STATES PATENT OFFICE

2,434,727

## METHOD OF PREPARING A PHOTOSENSITIVE BLOOD ALBUMIN LITHOGRAPHIC SOLUTION

Charles H. Van Dusen, Jr., Willoughby, Ohio, assignor to Addressograph-Multigraph Corporation, Cleveland, Ohio, a corporation of Delaware

No Drawing. Application August 7, 1944,  
Serial No. 548,515

2 Claims. (Cl. 95—7)

1

This invention relates to a photo-sensitive lithographic solution and to a method of preparing the same.

It has been common practice heretofore to utilize an aqueous egg albumin-ammonium dichromate solution as a photo-sensitive solution in the making of master lithographic or planographic printing plates by the photo-lithographic process. As is well known in the art, in this process the photo-sensitive solution is spread upon a zinc or other suitable metal plate which is then allowed to dry. The thus coated plate is then exposed, through a negative, to the action of an arc lamp, or other source of actinic light, which decomposes the ammonium dichromate and causes it to exert a so-called tanning or hardening effect upon the albumin. The plate is then coated with a so-called fatty or greasy lithographic printing ink and the unexposed or untanned or unhardened portions of the ammonium dichromate-albumin solution are thereupon washed off with water, whereupon, upon being treated with an aqueous planographic etching or dampening solution, the plate is ready for use.

While egg albumin is, in general, satisfactory for use in aqueous photo-sensitive lithographic printing solutions, it imparts to such solutions one objectionable characteristic, namely, a tendency to develop fungus mold growth.

I have found that blood albumin treated as hereinafter described, may advantageously be employed in photo-sensitive lithographic solutions in place of egg albumin and when so used is free from the objectionable tendency of egg albumin to promote fungus mold growth.

One difficulty, however, which I experienced and had to overcome in connection with the use of blood albumin in place of egg albumin in photo-sensitive lithographic solutions was the tendency of blood albumin to acquire an objectionable odor especially upon prolonged standing.

Another difficulty which I encountered, and had to overcome, in the use of blood albumin in photo-sensitive lithographic solutions was the presence of a certain amount of finely divided colloidal organic material in an aqueous solution of blood albumin and which had to be eliminated and the solution rendered substantially clear before it could be used as a photo-sensitive lithographic solution.

In connection with and as a part of the present invention, however, I have found that by treating an aqueous blood albumin solution according to a process which forms a part of the present invention, and which will be described presently,

2

the resulting aqueous blood albumin solution is rendered permanently substantially odorless as well as clear and free from suspended colloidal matter and affords a highly satisfactory photo-sensitive lithographic solution which has the advantage over egg albumin solutions in that it is substantially free from tendency toward fungus mold growth.

Accordingly, an object of the present invention is to afford a blood albumin photo-sensitive lithographic solution which is substantially free from tendency toward fungus mold growth while at the same time being substantially permanently odorless and clear or free from colloidally suspended matter.

Another object of the present invention is to afford a novel, simple and efficient method of preparing the new photo-sensitive lithographic solution.

Other and further objects of the present invention will be apparent from the following description and claims which, by way of illustration, illustrate the present invention and the principles thereof and what I now consider to be the best mode in which I have contemplated applying those principles. Other embodiments of the invention embodying the same or equivalent principles may be used and structural changes may be made as desired by those skilled in the art without departing from the present invention and the purview of the appended claims.

A typical process which may be followed in preparing the new clarified and deodorized blood albumin photo-sensitive lithographic solution is illustrated by the following example:

## Example

71 grams of a good grade of powdered blood albumin (Armour) are dissolved in 1500 cc. of water and the resulting solution is then filtered to remove suspended colloidal matter. For this purpose ordinary chemical filter paper is unsatisfactory in that such colloidal matter will pass directly through it. However, I have found that a filter aid composed essentially of a very finely divided diatomaceous earth, having a particle size of such, for example, as the filter aid known commercially as "J. M. Filtercel," affords a highly satisfactory filter in that it completely removes all suspended colloidal matter and affords a filtrate which is a clear aqueous blood albumin solution.

The thus filtered and clarified aqueous blood albumin solution is then deodorized by intimately mixing therein, with stirring, about 0.7 gram of

finely divided activated charcoal, whereupon the mixture is agitated for approximately thirty minutes to afford good contact of the finely divided activated charcoal particles with the aqueous blood albumin solution and resulting adsorption and removal of those substances in the solution which otherwise tend to impart an objectionable odor thereto.

The blood albumin-finely divided activated carbon mixture is then filtered again, by means of the finely divided diatomaceous earth filter aid referred to above, until the blackish cast imparted to the solution by the finely divided activated carbon is entirely removed and the solution is clear. Approximately 19 grams of a finely divided water-soluble dichromate such, for example, as finely divided ammonium dichromate  $(\text{NH}_4)_2\text{Cr}_2\text{O}_7$ , are then added to the solution, and stirred until dissolved therein, whereupon the hydrogen ion concentration or pH value of the resulting solution is adjusted by adding thereto a water solution of ammonia  $\text{NH}_4\text{OH}$  until the pH of the solution is not substantially more nor substantially less than 9.1.

In place of the ammonium dichromate specified in the foregoing example equivalent quantities of sodium dichromate or potassium dichromate, or various mixtures of these three water-soluble dichromates, may be used.

The resulting solution is a clear, yellowish and odorless and otherwise highly satisfactory photo-sensitive ammonium dichromate-blood albumin lithographic solution which is permanently free from tendency toward fungus mold growth. The solution being more yellowish than red in color indicates the presence of chromate as well as dichromate ions in the solution possibly due to some chromate salt in the dichromate or to the decomposition of some of the dichromate although as to the exact cause of this I am not certain. In any event, however, the term "dichromate" as used herein and as used hereinafter in the claims is intended to and does include not only water-soluble dichromate salts but also any water-soluble chromate salt which may be added to or be present in the solution as an impurity or as a result of the decomposition of the dichromate, or otherwise.

It will thus be seen from the foregoing description that the present invention affords a new and improved photo-sensitive lithographic solution having the desirable advantages and characteristics hereinbefore set forth, and others which are inherent in the invention, and also affords a new, simple and efficient method of preparing said solution, and thus accomplishes its intended objects and has the desirable ad-

vantages and characteristics hereinbefore pointed out and others which are inherent in the invention.

I claim:

- 5 1. The method of preparing a clear, odorless and fungus mold resistant photo-sensitive lithographic solution which comprises dissolving powdered blood albumin in water, filtering the resulting aqueous blood albumin solution to remove suspended colloidal matter, deodorizing the thus filtered aqueous blood albumin solution by intimately stirring finely divided activated carbon therein, filtering the aqueous blood albumin-finely divided activated carbon mixture to remove 10 the finely divided activated carbon therefrom, dissolving a water-soluble dichromate in the solution, and then adjusting the pH value of the resulting solution by adding an aqueous solution of ammonia thereto until the pH value of the solution is not substantially more nor substantially less than 9.1.
- 15 2. The method of preparing a clear, odorless, and fungus mold resistant photo-sensitive lithographic solution which comprises dissolving powdered blood albumin in water, filtering the resulting aqueous blood albumin solution to remove suspended colloidal matter therefrom, deodorizing the thus filtered aqueous blood albumin solution by intimately stirring finely 20 divided activated carbon therein, filtering the aqueous blood albumin-finely divided activated carbon mixture to remove the finely divided activated carbon therefrom, then dissolving ammonium dichromate in the resulting solution, and 25 then adjusting the pH value of the resulting solution by adding an aqueous solution of ammonia thereto until the pH value of the resulting solution is not substantially more nor substantially less than 9.1.
- 30 3. The method of preparing a clear, odorless, and fungus mold resistant photo-sensitive lithographic solution which comprises dissolving powdered blood albumin in water, filtering the resulting aqueous blood albumin solution to remove suspended colloidal matter therefrom, deodorizing the thus filtered aqueous blood albumin solution by intimately stirring finely 35 divided activated carbon therein, filtering the aqueous blood albumin-finely divided activated carbon mixture to remove the finely divided activated carbon therefrom, then dissolving ammonium dichromate in the resulting solution, and then adjusting the pH value of the resulting solution by adding an aqueous solution of ammonia thereto until the pH value of the resulting solution is not substantially more nor substantially less than 9.1.

40 CHARLES H. VAN DUSEN, JR.

#### REFERENCES CITED

The following references are of record in the file of this patent:

#### UNITED STATES PATENTS

| Number     | Name        | Date          |
|------------|-------------|---------------|
| 2,229,052  | Dell        | Jan. 21, 1941 |
| 51,181     | Hirsh       | Nov. 28, 1865 |
| 50 107,158 | Bourgade    | Sept. 6, 1870 |
| 2,189,380  | Littlefield | Feb. 6, 1940  |

#### OTHER REFERENCES

55 Eder, Ausfuhrliches Handbuch der Photograpie Band 4, 2 Teil (1926), entitled "Das Pigmentverfahren, U. S. W.", page 33. (Copy in Div. 7.)